

April 3, 1962

W. R. McKEIRNAN ET AL

3,028,288

FILM COATING FOR ELECTRON DEVICE ENVELOPES

Filed Sept. 30, 1959



INVENTORS

William R. McKeirnan  
Leonard D. Schwender  
BY Michael Hertz,  
ATTORNE

1

3,028,288

1  
FILM COATING FOR ELECTRON DEVICE  
ENVELOPES

William R. McKeirnan, Crosby, and Leonard D. Schwen-  
der, Emporium, Pa., assignors to Sylvania Electric  
Products Inc., a corporation of Delaware

Filed Sept. 30, 1959. Ser. No. 843,481  
2 Claims. (Cl. 156—86)

This invention relates to coatings on the exterior of elec-  
tron tubes and in particular to opaque coatings on glass  
envelopes enclosing photo-diodes.

In the prior art, opaque coatings had been applied either  
by hand brushing the coating material on the envelope  
or by spraying the material thereon resulting in coatings  
which might not display the desired opacity because of  
thinness in spots or in unnecessary heavy coating resulting  
from the use of excessive material. Both methods are  
sloppy because of the use of fluid materials.

It is an object of this invention to provide a coating  
on the exterior of an object, the coating to be applied  
without mess and to be of uniform characteristics, including  
uniform opaqueness and thickness throughout. As  
an illustration of the invention, the object coated is the  
envelope of a photo-diode.

The figure in the accompanying drawing represents a  
photo-diode with the coating of the invention.

The objects of the invention are effected by manufacturing  
the coating in the form of a self supporting film of  
even texture and thickness throughout and which incorporates  
a pigment within a soluble binder, and then, by  
application of a solvent for the binder in the film onto  
the envelope and contact of the envelope with the film,  
causing the film to wrap itself about the envelope.

A film suitable for covering photo diode glass envelopes  
may be made from a wide variation of proportions  
of materials, such as expressed in the following formulation:

|                       |             |            |    |
|-----------------------|-------------|------------|----|
| Toluene               | milliliters | 0 to 100   | 40 |
| Ethyl alcohol         | do          | 7 to 50    |    |
| Butyl carbitol        | do          | 0 to 10    |    |
| Ethyl cellulose N-200 | grams       | 1.5 to 15  |    |
| Triethanolamine       | milliliters | 0.4 to 0.6 |    |
| Graphite              | grams       | 30         |    |

The designation N-200 of the ethyl cellulose refers to  
the range of viscosities of the ethyl cellulose as set forth  
on page 5 of the Hercules Powder Company publication  
entitled "Ethyl Cellulose, Properties and Uses," copy-  
righted 1949.

The toluene and ethyl alcohol serve as solvents for the  
solid binder, such as ethyl cellulose. The butyl carbitol  
serves as a temporary plasticizer. The triethanolamine  
serves as an anti-oxidant for the cellulose.

A preferred suspension is made in accordance with the  
following formulation:

|                       |    |     |    |
|-----------------------|----|-----|----|
| Toluene               | ml | 100 | 60 |
| Ethyl alcohol         | ml | 50  |    |
| Butyl carbitol        | ml | 5   |    |
| Ethyl cellulose N-200 | gm | 10  |    |
| Triethanolamine       | ml | 0.5 |    |
| Graphite              | gm | 30  |    |

This suspension is thoroughly stirred in a glass container,  
then milled for sixteen hours in a ball mill to reduce the  
solids to a fine and even consistency. The suspension  
is then cast through a gate on a traveling trough onto  
a flat polished surface, as glass, into the form of a thin  
sheet of even thickness.

Preferably the trough travels about the surface with a  
four inch wide gate and the gate is raised above the surface  
to give a thickness of .0013" to the film.

2

Heat lamps are placed above the cast film to dry the  
film which film is then dampened with water to release  
it from the glass, from which it is stripped off by a suitable  
doctor blade. The film is then allowed to dry again.

The dry film now four inches wide and .0013" thick  
is then cut to suitable size to form leaves for application  
to the exterior of the photo-diode. If desired a window  
may be stamped out of each leaf prior to application of  
the leaf to the envelope, with the window in proper light  
registration with the photo-diode cathode or the window  
may be formed after the leaf has been applied to the envelope.  
The envelope has then applied to it a suitable  
solvent for the binder in the film, for example a mixture  
of the following five acetates:

N-amyl acetate  
2-methyl butyl acetate  
3-methyl butyl acetate  
4-methyl butyl acetate  
3-ethyl propyl acetate

The binder solvent may be applied to the envelope by  
dipping of the envelope in the solvent, by spraying the  
solvent on the envelope or by sponging of the envelope  
with the solvent. The solvent is quickly evaporative, but  
before it evaporates the envelope is brought into contact  
with the leaf whereupon, the solvent acts on the binder  
in the leaf to cause the leaf to wrap itself about the envelope.

While graphite was selected as the preferred coating  
for photo-diodes, another suitable opaque substance is  
ferric oxide black ( $Fe_3O_4$ ). In the above preferred formulation  
it was found that 24 grams of the ferric oxide  
could replace the 30 grams of graphite with equally good  
results.

In the drawing, the photo-diode is shown as having  
a glass envelope 12, coated with the coating 14 of the  
invention, a window 16 being provided in the coating  
for admission of light to the cathode. The coating on  
this tube besides being applied without mess, is uniform  
in thickness, in opaqueness and is neat in appearance  
since the coating has sharp parallel edges at the top and  
bottom of the cylindrical portions of the tube. Moreover  
the leaf is preferably made of a size to just wrap it-  
self around once about the envelope with the edges of  
the leaf in abutting relation.

What is claimed is:

1. The method of laminating a photo tube having a  
glass envelope with an opaque coating having a window  
therein, said method comprising manufacturing a self  
supporting thin opaque film with a window cut therein  
and comprised of an opaque pigmentation selected from  
the class of materials including graphite and ferric oxide  
black, said pigmentation being held in a soluble ethyl cel-  
lulose binder, wetting the exterior of the glass envelope  
with a solvent for the binder and bringing the envelope  
and self supporting film into contact whereby the film  
will wrap itself around the photo tube.

2. The method of laminating a photo tube having a  
glass envelope with a thin opaque film having a window  
cut out therein, said method comprising manufacturing  
a self supporting thin opaque film comprised of graphite  
held in a soluble ethyl cellulose binder, cutting a window  
in the film, wetting the surface of the photo tube with an  
organic solvent for the binder and contacting the film  
and tube, whereby the film wraps itself about the tube.

References Cited in the file of this patent

UNITED STATES PATENTS

70 2,425,351 Sharphouse Aug. 12, 1947  
(Other references on following page)

**3**  
UNITED STATES PATENTS

2,572,879 Morris et al. ----- Oct. 30, 1951  
2,686,269 Levitt ----- Aug. 10, 1954  
2,702,250 Miller ----- Feb. 15, 1955  
2,814,574 Friedman et al. ----- Nov. 26, 1957  
2,828,799 Harrison ----- Apr. 1, 1958  
2,986,671 Kerstetter et al. ----- May 30, 1961

## OTHER REFERENCES

Hackh's Chemical Dict., 3rd edition, page 166.  
Handbook of Material Trade Names—Zimmerman and  
5 Lavine, page 433. (Available Patent Office Tech. Li-  
brary.)